

May 28, 1974

YOSHIHIKO ABE

3,813,240

CORROSION-RESISTING STEEL

Filed June 21, 1972

2 Sheets-Sheet 1

FIG. 1



FIG. 1A



FIG. 3



May 28, 1974

YOSHIHIKO ABE

3,813,240

CORROSION-RESISTING STEEL

Filed June 21, 1972

2 Sheets-Sheet 2

FIG. 2



FIG. 2A



FIG. 4



1

3,813,240  
CORROSION-RESISTING STEEL  
Yoshihiko Abe, Tokyo, Japan, assignor to Mitsubishi  
Seiko Kabushiki Kaisha, Tokyo, Japan  
Filed June 21, 1972, Ser. No. 264,985  
Claims priority, application Japan, Mar. 3, 1972,  
47/21,554  
Int. Cl. C22c 37/10, 39/14  
U.S. Cl. 75—126 D 2 Claims

### ABSTRACT OF THE DISCLOSURE

The corrosion-resisting steel with superb resistance to pitting corrosion is manufactured of a microstructural stainless steel composed mainly of chromium or chromium added with at least one of nickel and manganese still containing 10 to 30 percent by weight of chromium and further having 2 to 10 percent by weight of one or more carbonitrides selected from the group of titanium, zirconium, niobium, tantalum and vanadium uniformly and finely dispersed therein.

### BACKGROUND OF THE INVENTION

The present invention relates to corrosion-resisting steels, and more particularly to steels with superb resistance to pitting corrosion and excellent corrosion resistance against any kind of acid solution.

In general, corrosion resistance is an indispensable characteristic for steels to be used in corrosive circumstances, and it is well known that many kinds of stainless steel have so far been developed for use under such circumstances. However, such stainless steels have neither sufficient pitting corrosion resistance nor corrosion resistance equally effective against all acid solutions, so the steels have to be selected according to the corrosive environment under which they are used.

### SUMMARY OF THE INVENTION

A principal object of the present invention is to provide corrosion-resisting steels without the drawbacks as inherent as in the conventional steels as abovementioned.

Another object of the present invention is to provide corrosion-resisting steels which have a superb pitting corrosion resistance quality as unobtainable in the conventional steels.

A further object of the present invention is to provide corrosion-resisting steels which have a matrix of cheap ferrite structure.

Still further object of the present invention is to provide corrosion-resisting steels which show excellent corrosion resistance to various acid solutions.

A steel according to the present invention is characterized by the fact that it is manufactured by adding into a conventional stainless steel some alloy components hav-

2

ing specific carbonitrides dispersed therein uniformly and finely beyond a certain degree of concentration.

### BRIEF DESCRIPTION OF THE DRAWINGS

These and other objects of the present invention will become more apparent to those skilled in the art when considered in reference to the following detailed description in the light of the accompanying drawings wherein:

FIGS. 1 and 1(a) show the result of tests, in which the effect of molybdenum quantity contained in the steel according to the present invention was tested in 2% and 35% hydrochloric acid solutions;

FIGS. 2 and 2(a) show the results of tests, in which the effect of aluminum quantity contained in the steel according to the present invention was tested in 33% and 65% nitric acid solutions;

FIG. 3 shows the test result of six samples in Table 2 comparing their corrosion resistances under several conditions of heat treatment; and

FIG. 4 shows a quantitative relation of copper and titanium causing an improvement on corrosion resistance in the test shown in FIG. 3.

### DETAILED DESCRIPTION OF INVENTION

The steel according to the present invention is produced by a process in which the molten steel containing much excess carbon compared with oxygen, nitrogen and sulphur contents are added with some elements to form carbonitrides so that these elements preferentially react with carbon, and the thus-obtained solid carbides are uniformly dispersed and precipitated together with the solid nitrides and the dispersed carbonitrides must be stable even under hot and corrosive conditions thereafter.

As elements to precipitate such homogeneous dispersoid particle and to produce stable carbonitrides in a hot and corrosive environment, titanium, zirconium, niobium, tantalum and vanadium are given. One or more elements of them constitute such sole or complex carbonitrides. In these carbonitride dispersion-strengthened materials, size of dispersoid particles, homogeneity and dispersed quantity are the most important factors to affect the characteristics.

It was found out that adding 0.2% or less phosphorus is effective to improve the homogeneity and preferential forming of boronnitride in the molten steel by adding 0.2% or less boron is desirable.

From the foregoing explanation, it is evident that the steel according to the present invention can be produced industrially. The following explanation relates to the kinds and necessary quantity of carbonitrides evenly dispersed into the steel according to the present invention, and also components and necessary quantity of the matrix in which carbonitrides are dispersed.

The result of the tests having investigated the effect of quantity of dispersed carbonitride and quantity of chromium in the matrix for pitting corrosion in 5% ferric chloride solution (pH 1.25) is shown in Table 1.

TABLE 1

| Sample number | Element(s) | Dispersed carbonitride |       | Components in matrix (percent) |    | Corrosion appearance     |
|---------------|------------|------------------------|-------|--------------------------------|----|--------------------------|
|               |            | Percent                | Cr    | Structure                      | Cr |                          |
| 1             | Ti         | 5.1                    | 5.08  | Cr ferrite                     | —  | Terribly uniform attack. |
| 2             | Ti         | 4.7                    | 8.7   | do                             | —  | Do.                      |
| 3             | Ti         | 3.2                    | 10.43 | do                             | —  | Pitting.                 |
| 4             | Ti plus Nb | 6.1                    | 13.1  | Cr-Mo ferrite                  | —  | Do.                      |
| 5             | Zr         | 5.4                    | 15.6  | Cr ferrite                     | —  | Do.                      |
| 6             | Ti plus V  | 7.5                    | 17.6  | Cr-Mn austenite                | —  | Do.                      |
| 7             | Ti         | 5.0                    | 18.3  | Cr-Ni austenite                | —  | Not pitting.             |
| 8             | Zr plus V  | 3.9                    | 17.0  | Cr-Ni-Mn austenite             | —  | Pitting.                 |
| 9             | Ti         | 3.5                    | 17.9  | Cr-Mo ferrite                  | —  | Not pitting.             |
| 10            | Ti plus Nb | 2.3                    | 17.2  | do                             | —  | Do.                      |
| 11            | Ti         | 1.4                    | 18.4  | do                             | —  | Localized pitting.       |
| 12            | —          | 0                      | 17.9  | Cr ferrite                     | —  | Uniform attack.          |
| 13            | —          | 0                      | 18.7  | Cr-Ni austenites               | —  | Localized pitting.       |
| 14            | Ti plus Ta | 4.5                    | 22.9  | Cr-Ni ferrite-austenite        | —  | Not attack.              |
| 15            | Ti         | 4.6                    | 24.5  | Cr ferrite                     | —  | Do.                      |
| 16            | Ti         | 4.7                    | 24.5  | Cr-Ni austenite                | —  | Do.                      |
| 17            | Ti plus Zr | 3.9                    | 25.1  | Cr-Mn austenite                | —  | Do.                      |

Table 1 shows that it is necessary to add 10% or more chromium into the matrix to completely prevent corrosion of the steel regardless the micro-structure of the matrix.

Furthermore it is comprehensible that any kind of carbonitride increases its resistance to pitting corrosion, if 2.0% or more of sole carbonitride of titanium or zirconium, or complex carbonitride of titanium and niobium, titanium and vanadium, or zirconium and tantalum are dispersed into the matrix containing 10% or more chromium. Therefore, in the steel according to the present invention, it is inevitable to precipitate dispersely 2% or more carbonitride abovementioned into the steel.

If the matrix of steel contains 10% or more chromium, any kind of existing stainless steels can be applied, whether the structure of matrix is ferrite containing chromium as

The corrosion resistance of the steel of the present invention to sulfuric acid can be remarkably increased by containing three elements, nickel, copper and titanium together in the matrix.

FIG. 3 represents a comparison of corrosion resistances to 5% sulfuric acid solution of six samples having different quantities of nickel, copper and titanium in the matrix as shown in Table 2. It is found out that adding only two elements combined, copper and nickel, copper and titanium or nickel and titanium does not show marked effect to corrosion resistance, but the ferritic steel containing three elements, nickel, copper and titanium, together has excellent corrosion resistance under the condition of 500°-800° C. heat treatment and the austenitic steel containing three elements above mentioned, has also strong corrosion resistance under any condition of heat treatment.

TABLE 2

| Sample number | Dispersed carbonitride<br>Element(s) | Percent | Components in matrix, percent |      |       |       | Matrix structure     |
|---------------|--------------------------------------|---------|-------------------------------|------|-------|-------|----------------------|
|               |                                      |         | Ni                            | Cr   | Cu    | Ti    |                      |
| 17            | Ti                                   | 5.0     | 8.2                           | 19.7 | ----- | 0.8   | Austenite.           |
| 18            | Ti plus Zr                           | 3.9     | -----                         | 16.1 | 0.65  | 1.00  | Ferrite.             |
| 19            | Ti plus Ta                           | 4.3     | 1.4                           | 17.3 | 0.74  | ----- | Do.                  |
| 20            | Ti                                   | 3.3     | 1.6                           | 17.3 | 1.31  | 1.20  | Do.                  |
| 21            | Ti plus Nb                           | 4.0     | 8.8                           | 18.3 | 1.34  | 0.75  | Austenite (Cr-Ni).   |
| 22            | Ti                                   | 3.8     | 3.8                           | 17.1 | 1.64  | 0.83  | Austenite (Cr-Ni-Mn) |

a main component of alloy, or ferrite-austenite or austenite containing one or two elements of chromium, nickel and manganese. In the steel according to the present invention, however, maximum quantities of dispersed carbonitride and chromium are limited from the production engineering standpoint, and it is desired that quantity of carbonitride is limited to 10% or less owing to fluidity and quantity of chromium is limited to 30% or less due to plasticity.

The corrosion resistance of the steel according to the present invention to acid solution containing chloridion can be remarkably improved by containing molybdenum in the matrix.

FIGS. 1 and 1(a) shows the variation of corrosion rate of the steel according to the present invention in hydrochloric acid solutions of different concentrations against the quantitative change of molybdenum content in the matrix. The effect of molybdenum appears conspicuously about 0.7% and saturates about 4%. Therefore quantity of molybdenum content may be limited to 0.5-5.0%.

It is remarked additionally that the effect of added molybdenum is not influenced by quantity of chromium or carbonitride as far as the steel of the present invention is concerned.

Similarly the corrosion resistance of the steel according to the present invention to nitric acid can be improved by adding aluminum in the matrix. FIGS. 2 and 2(a) represent the variation of corrosion rate of the steel against quantities of aluminum in its matrix containing 18% and 25% chromium respectively, and having 3.5-5.0% various carbonitrides dispersed.

In both cases, it is found out that the effect appears at 0.2% or more and saturates at 0.5% or more.

Hence, considering the defect of aluminum for plastic deformation, quantity of aluminum may be limited to 0.2-1.0% in maintaining its effect sufficiently.

In the steel containing three elements, nickel, copper and titanium, together, quantity of nickel shall be preferably more than 1.5 times that of copper to prevent hot brittleness due to copper. FIG. 4 shows the domain of corrosion resistance rate of the steel against various quantities of copper and titanium, keeping quantity of nickel content 1.5 times that of copper. Minimum quantities to improve the corrosion resistance are 0.4% copper and 0.2% titanium.

It has been made clear that the corrosion resistance is improved as added elements increase, and it is much improved with 0.9% copper and 0.6% titanium added, but the resistant property saturates over that quantity.

Therefore, for corrosion-resisting steel to sulfuric acid, ferrite-austenitic steel and austenitic steel containing 10-30% chromium and at least 3% nickel, shall have 2-10% said carbonitride dispersed into the matrix containing 0.4-2.0% copper and 0.2-1.5% titanium, and other stainless steel shall have the same quantity of carbonitride dispersed into the matrix containing 0.6-3.0% nickel additionally. In case that the corrosion resistance to hydrochloric acid or nitric acid is to be supplemented, one or two elements of 0.5-5.0% molybdenum and 0.2-1.0% aluminum shall be added.

The following examples will serve to illustrate the excellent corrosion resistance of the steel according to the present invention.

#### EXAMPLE 1

SUS24B containing 16-18% chromium as a main component and the steel according to the present invention in which 3.2% by weight of complex carbonitride of titanium and niobium was dispersed, were immersed in acid solution containing 5.0% chloridion. Pitting corrosion appeared on SUS24B in three days, but no corrosion was found on the invented steel after ten days.

Test pieces of 25 x 5 x 50 mm. were cut off from the two steels and they were immersed in boiling solution of 10% sulfuric acid containing 10% copper sulphide for one hour.

Then SUS24B got terrible corrosion over the entire surface and 40% of it was dissolved, while the invented steel had no remarkable corrosion and dissolution rate was less than 0.1%.

#### EXAMPLE 2

SUS42B, which contains 24-26% chromium, 19-22% nickel as main alloy components, is the highest grade stainless steel having excellent corrosion resistance.

The steel according to the present invention which has carbonitride containing 4.0% titanium carbide as a main component, dispersed in the matrix having only 2% molybdenum besides the same quantity of chromium as SUS42B, was tested for corrosion resistance comparing with SUS42B in acid solution containing chloridion.

As shown in Table 3, the invented steel proved to have extraordinarily excellent corrosion resistance judging from both corrosion appearance and corrosion rate, and the difference was obvious in sodium chloride solution.

TABLE 3

| Corrosive solution                                           | Invented steel     | SUS-42B                  | Corrosion rate g./m. <sup>2</sup> /day (corrosion appearance) |
|--------------------------------------------------------------|--------------------|--------------------------|---------------------------------------------------------------|
| 10% FeCl <sub>3</sub> ·6H <sub>2</sub> O solution (pH 1.25)  | 0.3 (Not pitting)  | 8.2 (Localized pitting)  |                                                               |
| 7.5% FeCl <sub>3</sub> ·6H <sub>2</sub> O solution (pH 1.25) | 0.18 (Not pitting) | 6.8 (Localized pitting)  |                                                               |
| 5% FeCl <sub>3</sub> ·6H <sub>2</sub> O solution (pH 1.25)   | 0.06 (Not pitting) | 0.09 (Not pitting)       |                                                               |
| 6.1% NaCl solution (pH 2.5)                                  | 0.08 (Not pitting) | 9.48 (Localized pitting) |                                                               |

#### EXAMPLE 3

The steel according to the present invention which has carbonitride containing 3.7% titanium carbide as a main component, dispersed in the matrix containing 18% chromium, 1.2% nickel, 0.75% copper, 0.25% titanium, 2.0% molybdenum, was heat-treated at 650° C. and tested for corrosion resistance in various acid solutions comparing with 18% chromium, 8% nickel stainless steel (SUS27B) most commonly used.

The test result shown in Table 4 reveals that the steel of the present invention is slightly inferior to SUS27B in corrosion resistance to nitric acid, but it is superior in corrosion resistance to sulfuric acid, and moreover it has specific high corrosion resistance in acid solution containing hydrochloric acid and chloridion.

TABLE 4

| Corrosive solution                               | Corrosion rate (g./m. <sup>2</sup> /hr.) |                                          |                       |
|--------------------------------------------------|------------------------------------------|------------------------------------------|-----------------------|
|                                                  | Invented steel (no aluminum contained)   | Invented steel (0.4% aluminum contained) | SUS27B                |
| 2% hydrochloric acid solution (room temperature) | 0.87                                     | 0.85                                     | 2.2                   |
| 2% hydrochloric acid solution (boiling)          | 31.2                                     | 31.5                                     | 54.3                  |
| 2% hydrochloric acid solution (boiling)          | 780                                      | 774                                      | 8,180                 |
| 3% hydrochloric acid solution (room temperature) | 29.9                                     | 30.7                                     | 429                   |
| 3% nitric acid solution (boiling)                | 0.14                                     | 0.08                                     | 0.07                  |
| 6% nitric acid solution (boiling)                | 0.82                                     | 0.22                                     | 0.22                  |
| 5% sulfuric acid solution (boiling)              | 23                                       | 20.5                                     | 179                   |
| 90% sulfuric acid solution (40° C.)              | 0.17                                     | 0.15                                     | 0.56                  |
| 6.1% NaCl solution (room temperature)            | 3.3×10 <sup>-3</sup>                     | 3.3×10 <sup>-3</sup>                     | 3.60×10 <sup>-3</sup> |

Even in this case, the steel according to the present invention, if 0.4% aluminum added, has the same corrosion resistance to nitric acid as SUS27B.

What is claimed is:

1. A corrosion-resistant steel having a microstructure consisting essentially of 2-10% by weight of a carbonitride of one or more elements selected from the group consisting of titanium, zirconium, niobium, tantalum and vanadium uniformly and finely dispersed in a stainless steel consisting essentially of 10-30% of chromium, an effective amount up to 0.2% of phosphorus, an effective amount up to 0.2% boron and the balance being iron.

2. A corrosion resisting steel having a microstructure consisting essentially of 2-10% by weight of a carbonitride of one or more elements of titanium, zirconium, niobium, tantalum and vanadium uniformly and finely dispersed into the stainless steel, 10-30% by weight of chromium, one or more elements of less than 0.2% boron or phosphorous, 0.5-5.0% by weight of molybdenum, 0.2-1.0% by weight of aluminum, 0.4-2.0% by weight of copper, 0.6-3.0% by weight of nickel, 0.2-1.5% by weight of titanium, and the balance being iron.

#### References Cited

##### UNITED STATES PATENTS

|           |         |                |        |
|-----------|---------|----------------|--------|
| 3,690,869 | 9/1972  | Zelenodolskaya | 75-124 |
| 3,152,934 | 10/1964 | Lula           | 75-124 |
| 3,365,343 | 1/1968  | Vordahl        | 75-124 |
| 3,674,469 | 7/1972  | Stewart        | 75-124 |

HYLAND BIZOT, Primary Examiner

U.S. Cl. X.R.

75-126 F, 126 D, 124, 125